

[54] METHOD FOR IMPROVING THE FIRE  
RESISTANCE OF NYLON AND POLYESTER  
FABRICS

[75] Inventor: Jay C. Chapin, Marblehead, Mass.

[73] Assignee: Ventron Corporation, Beverly,  
Mass.

[22] Filed: June 19, 1972

[21] Appl. No.: 264,342

[52] U.S. Cl..... 117/136, 117/137, 117/138.8 N,  
117/138.8 F, 252/8.1

[51] Int. Cl..... C09d 5/18

[58] Field of Search..... 117/136, 138.8 N,  
117/138.8 F, 139.5 CQ, DIG. 3, 137;  
252/8.1; 106/15 FP

[56] References Cited

UNITED STATES PATENTS

2,436,181 2/1948 Rosser ..... 117/136

|           |        |                     |             |
|-----------|--------|---------------------|-------------|
| 2,922,726 | 1/1960 | Morretti et al..... | 117/137     |
| 3,600,219 | 8/1971 | Reuter et al.....   | 117/138.8 F |
| 3,669,725 | 6/1972 | Nachbur et al.....  | 117/136     |
| 3,692,559 | 9/1972 | Powell .....        | 117/138.8 F |

OTHER PUBLICATIONS

Schmerda, J. Soc. Chem. Ind., 36, 942, Aug. 31, 1917.

Primary Examiner—William D. Martin  
Assistant Examiner—Theodore G. Davis  
Attorney—J. Harold Boss

[57] ABSTRACT

The resistance to burning and flame propagation of synthetic textile fabrics, such as nylon and polyester is improved by treatment with an aqueous solution of formaldehyde and ammonium thiocyanate and drying.

2 Claims, No Drawings

**METHOD FOR IMPROVING THE FIRE  
RESISTANCE OF NYLON AND POLYESTER  
FABRICS**

The invention relates to a method for treating synthetic textile fabrics, such as nylon and polyester, to improve their resistance to burning and flame propagation.

In accordance with the method of the invention the synthetic fabric is saturated with an aqueous solution containing from about 6 to 24 percent by weight of formaldehyde and about 20 to 28 percent by weight of ammonium thiocyanate both by weight based on the dry weight of the fabric. Excess solution is removed and the treated fabric dried at a temperature between room temperature and 275°F. to cause the formaldehyde and ammonium thiocyanate to react to form a polymer. Unreacted material is removed by rinsing with water. The reaction product is resistant to removal by drying cleaning and laundering procedures.

The reaction of ammonium thiocyanate with formaldehyde has been previously described by Schmerda, J. Soc. Chem. Ind., 36,942. When reacted with equimolar quantities of formaldehyde and ammonium thiocyanate in concentrated aqueous solution yellow amorphous compounds are obtained which have no definite melting points. With the use of different ratios of formaldehyde and ammonium thiocyanate different types of resins have been obtained.

When an aqueous solution of formaldehyde and ammonium thiocyanate is prepared and permitted to stand the pH of the solution gradually decreases as shown in Table I.

**Table I**

| Time   | Change in pH in ageing solution of 1:1 Molar ratio of $\text{CH}_2\text{O}$ and $\text{NH}_4\text{SCN}$ |      |
|--------|---------------------------------------------------------------------------------------------------------|------|
|        | Temp.                                                                                                   | pH   |
| 5 mins | 10°C                                                                                                    | 3.5  |
| 10     | 13                                                                                                      | 2.4  |
| 20     | 13                                                                                                      | 1.8  |
| 25     | 18                                                                                                      | 1.8  |
| 30     | 19                                                                                                      | 1.1  |
| 35     | 20                                                                                                      | 0.9  |
| 40     | 22                                                                                                      | 0.7  |
| 45     | 23                                                                                                      | 0.45 |
| 50     | 25                                                                                                      | 0.30 |
| 55     | 26                                                                                                      | 0.20 |
| 60     | 27                                                                                                      | 0.15 |

With a ratio of  $\frac{1}{2}\text{M}$   $\text{CH}_2\text{O}$ :1M  $\text{NH}_4\text{SCN}$  the change in pH of the solution was similar. With a ratio of 2M  $\text{CH}_2\text{O}$ /1M  $\text{NH}_4\text{SCN}$  a drop of pH was also noted. The pH drop of the solution could be retarded by keeping the solution below 10°C. After an hour with all three solutions at a temperature of about 27°C a precipitation of solid polymer had commenced. At the end of 24 hours the weight of solid polymer from the 3 solutions was determined. See Table II.

**Table II**

| Ratio                                                                    | Yield From Reaction of $\text{CH}_2\text{O}$ and $\text{NH}_4\text{SCN}$ |                   |
|--------------------------------------------------------------------------|--------------------------------------------------------------------------|-------------------|
|                                                                          | Weight of Polymer                                                        | Weight of Polymer |
| 1M $\text{CH}_2\text{O}$ : 1M $\text{NH}_4\text{SCN}$                    | 48 grams                                                                 |                   |
| 2M $\text{CH}_2\text{O}$ : 1M $\text{NH}_4\text{SCN}$                    | 64 grams                                                                 |                   |
| $\frac{1}{2}\text{M}$ $\text{CH}_2\text{O}$ : 1M $\text{NH}_4\text{SCN}$ | 25 grams                                                                 |                   |

These polymers are insoluble in chlorinated hydrocarbons such as are used for dry cleaning and also are not soluble in caustic solution.

**Example I**

Because of the rapidity with which these polymers form treatments of fabrics must be made shortly after solution or provision made for keeping the treating solution at a temperature of 10°C or lower. Within 5 minutes of making up a 1:1 molar solution containing 76 grams of  $\text{NH}_4\text{SCN}$ , 86 grams of 37%  $\text{CH}_2\text{O}$  and 100 grams of water a 6.5 oz/yd<sup>2</sup> polyester drapery fabric of the polyester/Dacron type was padded through the treating solution and excess solution was squeezed out until the wet pickup, based on the original dry weight of the fabric was 75 percent. After treatment of the fabric was dried 5 minutes at 250°F. in a hot air circulating oven. After drying the fabric was weighed and then rinsed of unreacted material and weighed again. The rinsing step removed about half of the dry add-on deposited on the fabric. The rinsed fabric after drying when tested in accordance with Flame Retardant Method 34-1969 AATCC was found to be immediately self extinguishing after removal of the ignition source. A glass thread was not stitched into the fabric as the method suggests for thermo plastic fabrics. Also little smoke generation was noted and the ignited fabric did not drip during a 12 sec. ignition exposure. This fabric was also self extinguishing after one Tide washing in an automatic home washing machine.

**EXAMPLE II**

45 A treating solution in a 2 to 1 molar ratio was made up containing 166 grams of 37%  $\text{CH}_2\text{O}$  solution and 76 grams of  $\text{NH}_4\text{SCN}$  and 17 grams of water. Polyester fabric was treated from this solution in a manner similar to that of Example I. This fabric was also immediately self extinguishing after removal of the 12 sec. ignition flame. The handle of this fabric was slightly stiff after rinsing.

**EXAMPLE III**

55 A third piece of polyester fabric was treated from a solution containing a 1/2 to 1 molar ratio of  $\text{CH}_2\text{O}$  and 76 grams of  $\text{NH}_4\text{SCN}$  and 140.5 grams of water. The polyester was treated from this solution in a manner similar to that of the treatment in Example I. The rinsed fabric after drying was also self extinguishing after 12 sec. ignition. After one Tide washing this fabric after 12 sec. ignition exposure had an afterflame of 18 sec. and its burning behavior was similar to the untreated fabric. The results of these 3 examples are summarized in Table III.

Table III

| Example | Ratio                                                    | Reaction of various molar ratios of $\text{CH}_2\text{O}$ and $\text{NH}_4\text{SCN}$ on polyester |                               |                              |
|---------|----------------------------------------------------------|----------------------------------------------------------------------------------------------------|-------------------------------|------------------------------|
|         |                                                          | Dry add-on o.w.f.* after drying                                                                    | Dry add-on o.w.f. after rinse | After flammimg AATCC 34-1969 |
| I       | 1M $\text{CH}_2\text{O}$<br>1M $\text{NH}_4\text{SCN}$   | 19.3                                                                                               | 9.5                           | -0-                          |
| II      | 2M $\text{CH}_2\text{O}$<br>1M $\text{NH}_4\text{SCN}$   | 26.2                                                                                               | 22.4                          | -0-                          |
| III     | 1/2M $\text{CH}_2\text{O}$<br>1M $\text{NH}_4\text{SCN}$ | 18.3                                                                                               | 5.6                           | -0-                          |

\*o.w.f. original weight of fabric

#### EXAMPLE IV

A treating solution was made up containing 80 grams  $\text{NH}_4\text{SCN}$ , 128 grams of 37%  $\text{CH}_2\text{O}$  and 196 grams of water. This provided a solution containing about 12 percent by weight of formaldehyde and about 20 percent by weight of  $\text{NH}_4\text{SCN}$ . An 8.0 oz/yd<sup>2</sup> nylon upholstery fabric treated from this solution had a wet pickup based on the original weight of the fabric of 95%. The upholstery fabric was dried in a hot air circulating oven for 5 mins. at 275°F. This fabric was immediately self extinguishing after 12 sec. ignition in accordance with Method 34-1969 AATCC. (A glass thread was not stitched into the fabric as the method suggests for thermoplastic fabrics). This fabric also did not drip during ignition and there was little smoke observed.

I claim:

1. The method for improving the resistance to burning and flame propagation of synthetic textile material

selected from the group consisting of nylon and polyester, which comprises saturating the textile material with an aqueous solution containing from about 6 to 24 percent by weight of formaldehyde and about 20 to 28 percent by weight of ammonium thiocyanate based upon the dry weight of the textile material, drying the treated textile material at a temperature between room temperature and about 275°F. thereby causing the formaldehyde and  $\text{NH}_4\text{SCN}$  to react to form a polymer, and removing unreacted material from the treated textile material by rinsing with water.

2. The method as claimed by claim 1 wherein the amount of formaldehyde in the aqueous treating solution is about 20 percent by weight of ammonium thiocyanate based upon the dry weight of the textile material and about 12 percent by weight of formaldehyde based on the dry weight of the textile material.

\* \* \* \* \*

35

40

45

50

55

60

65